



US008689378B2

(12) **United States Patent**  
**Khambete**

(10) **Patent No.:** **US 8,689,378 B2**  
(b5) **Date of Patent:** **Apr. 8, 2014**

(54) **CUSHION STRUCTURE AND CONSTRUCTION**

(75) Inventor: **Surendra S. Khambete**, West Bloomfield, MI (US)

(73) Assignee: **IndraTech LLC**, West Bloomfield, MI (US)

(\*) Notice: Subject to any disclaimer, the term of this patent is extended or adjusted under 35 U.S.C. 154(b) by 901 days.

(21) Appl. No.: **12/605,862**

(22) Filed: **Oct. 26, 2009**

(65) **Prior Publication Data**

US 2011/0094038 A1 Apr. 28, 2011

(51) **Int. Cl.**

*A47C 16/00* (2006.01)  
*B68G 5/00* (2006.01)

(52) **U.S. Cl.**

USPC ..... **5/655.6**; 5/653; 5/655.9; 5/731; 5/408; 5/948; 5/952

(58) **Field of Classification Search**

USPC ..... 5/652, 653, 655.6, 655.9, 731, 408, 5/948, 952, 969; 428/74, 223, 76, 156, 428/171, 172, 175; 442/381, 387; 112/470.27, 475.14

See application file for complete search history.

(56) **References Cited**

U.S. PATENT DOCUMENTS

2,403,043 A \* 7/1946 Bowersox ..... 5/696  
3,335,435 A \* 8/1967 Marsh et al. ..... 5/652  
4,207,636 A 6/1980 Ceriani  
4,618,531 A 10/1986 Marcus

|                   |         |                  |         |
|-------------------|---------|------------------|---------|
| 4,940,502 A       | 7/1990  | Marcus           |         |
| 5,169,580 A       | 12/1992 | Marcus           |         |
| 5,272,000 A       | 12/1993 | Chenoweth et al. |         |
| 5,294,392 A       | 3/1994  | Marcus           |         |
| 5,552,205 A *     | 9/1996  | Lea .....        | 428/74  |
| 6,155,647 A       | 12/2000 | Albecker, III    |         |
| 7,166,547 B2      | 1/2007  | Tilton et al.    |         |
| 7,216,936 B2      | 5/2007  | Peterson         |         |
| 2006/0175883 A1   | 8/2006  | Neustat          |         |
| 2007/0293113 A1 * | 12/2007 | Ogle .....       | 442/414 |

OTHER PUBLICATIONS

Otis Bed Manufacturing, Futons, "Moonshadow, Elite plush polyester wrapped foam futon," [www.otisbed.com/moonshadow.php](http://www.otisbed.com/moonshadow.php), May 29, 2009.

Polyurethane Foam Association, "Joint Industry Foam Standards and Guidelines," Sections 0.0 through 15.0, Appendixes A1.0 through A4.0, published Jul. 1994, [www.pfa.org/jifsg/jifsgs0.html](http://www.pfa.org/jifsg/jifsgs0.html).

\* cited by examiner

*Primary Examiner* — Robert G Santos

*Assistant Examiner* — David E. Sosnowski

(74) *Attorney, Agent, or Firm* — Carlson, Gaskey & Olds P.C.

(57) **ABSTRACT**

A cushion assembly includes an aesthetic cover having a perimeter panel providing a perimeter height. Spaced apart cover panels extend between the perimeter panels. The perimeter and cover panels together provide a cushion cavity. A cushion includes randomly oriented fibers bonded to one another to provide a core of a batt that has opposing surfaces. The batt includes manufactured, tufted and desired design heights. A tuft extends through the cushion to the opposing surfaces to maintain the cushion in the tufted height, which is less than the manufactured height. The cushion is provided at the desired design height with the tufted cushion arranged within the cushion cavity. The tufted height is generally less than the desired design height.

**10 Claims, 2 Drawing Sheets**





FIG. 1



FIG. 5



FIG. 7



FIG. 8



## 1

## CUSHION STRUCTURE AND CONSTRUCTION

## BACKGROUND

This disclosure relates to a cushion structure, assembly and its construction for comfort applications, including seating and bedding utilizing polyester fiber as one filler material.

A typical cushion assembly used in seating applications includes an aesthetic cover surrounding a soft and resilient filler material such as polyurethane foam, springs and the like. Most cushions are constructed with material which provides a desired support and comfort to the user. Polyester fiber toppers are sometimes used on top and side of the cushion assembly on which a user may sit to provide a better "hand," which is a desired feel. An additional wrap is occasionally used to provide a desired function such as to provide improved resistance against flammability. The wrapped and/or padded core structure, usually made up of polyurethane foam is inserted into an aesthetic cover. The foam core is generally the same dimensions as the cover or very slightly larger than the cover.

The feel of foam cushions is very customizable. This is done by changing the foam chemistry for a given density. One measurement of "feel" for a cushion is the Indentation Load Deflection, ILD, which is determined using industry guidelines. The ILD is the amount of pounds (measured as resistant force) required to compress a 4 inch thick, 15 inch×15 inch sample to 3 inches (or 25% of original height). For example, a typical 4 inch tall polyurethane foam cushion having a density (in pounds per cubic foot, or "pcf") of 1.0 pcf has an ILD of 30. In addition due to processing and chemistry changes this is tunable within a range of 10-40 ILD; a density of 1.2 pcf is tunable to 20-50 ILD; and so on.

A given foam cushion must also exhibit an acceptable comfort or "support factor," typically in the range of 1.7-3.0. The support factor calculated by dividing the force required to compress a 4" sample to 65% of its height by the force required to compress to 25% of its height; i.e. comfort factor=(ILD @ 65%)/(ILD @ 25%) In addition to comfort, a standard foam cushion must survive industry durability tests over several thousand cycles during which the foam cushion must substantially maintain its height and shape while maintaining the support factor. Polyurethane foam cushions are highly tunable in that a foam material can be easily selected to provide a desired density, ILD and support factor, which in turn provides the durability for a given application. For polyester fiber cushions, the ILD is very closely tied to the density and such fiber cushions are not easily tuned to provide both comfort and durability. To provide better durability fiber cushions must be made very dense but that is generally not acceptable as comfortable for the end user.

Foam is generally very resilient and tunable but the chemistry is such that in its native state it is very highly flammable, further the process of making foam is considered harmful to the environment. Several attempts to replace foam with polyester fiber have resulted in different formed, thermo-bonded or loose fiber constructions, but none have been able to achieve desired comfort and performance sufficient for broad commercial viability due to the difficulty in tuning. Loose fibers or thermo-bonded fibers are sometimes used in outdoor cushion applications to provide improved long-term resiliency over foam. The fibers are loosely arranged relative to one another in an unconnected fashion, permitting the fibers to shift uninhibited within the cover. Such outdoor cushions are not very durable and as such not suitable for conventional seating and bedding applications.

## 2

Tufting has been used to secure multiple layers to one another or provide an aesthetically pleasing exterior cover. Often, the tufts are visible through the cover. For example, tufting is used in futons to secure the multiple layers to one another and the exterior cover. The exterior cover is arranged rather loosely about the layers.

## SUMMARY

10 A cushion assembly includes an aesthetic cover having a perimeter panel providing a perimeter height. Spaced apart cover panels extend between the perimeter panels. The perimeter and cover panels together provide a cushion cavity. A cushion includes randomly oriented fibers bonded to one another to provide a core of a batt that has opposing surfaces. In one disclosed example, the fibers are polyester and include an average length randomly oriented in three dimensions. The core has a thickness that is greater than the average length to accommodate the average length in all three dimensions.

15 20 The batt includes manufactured, tufted and desired design heights. A tuft extends through the cushion to the opposing surfaces to maintain the cushion in the tufted height, which is less than the manufactured height. The cushion is provided at the desired design height with the tufted cushion arranged within the cushion cavity. The tufted height is generally less than the desired design height.

25 30 These and other features of the disclosure can be best understood from the following specification and drawings, the following of which is a brief description.

## BRIEF DESCRIPTION OF THE DRAWINGS

35 FIG. 1 is a perspective view of an example cushion assembly.

40 FIG. 2 is a cross-sectional view of a prior art foam cushion at a manufactured height.

45 FIG. 3A is a side elevational view of a randomly oriented fiber cushion having a manufactured height for the same cushion application as the foam cushion illustrated in FIG. 2.

50 FIG. 3B is a schematic view of the randomly oriented fibers interlinked to one another with binder material.

55 FIG. 4 is a cross-sectional view of the fiber cushion illustrated in FIG. 3A that has been tufted.

FIG. 5 is a cross-sectional view of a cushion having topper layers.

FIG. 6 is a side elevational view of an example tuft.

FIG. 7 is a cross-sectional view of the cushion illustrated in FIG. 5 with a wrap and inserted into a cover.

55 FIG. 8 is a side elevational view of a cushion assembly according to the disclosure compared to a cushion assembly using the foam illustrated in FIG. 2 for the same cushion application.

## DETAILED DESCRIPTION

55 A cushion assembly 10 is schematically illustrated in FIG. 1. The cushion assembly 10 includes a cover 11 having a perimeter panel 12 joined to opposing cover panels 14 at edge 20. Typically, the perimeter and cover panels 12, 14 are sewed to one another at the adjoining edges 20 using a welting. A closure 18, such as a zipper, edge tape or hook-and-loop fastener, is provided at a seam 16 to permit insertion of a cushion into a cavity provided within the cover 11.

60 65 FIG. 2 schematically illustrates a typical foam cushion 22 having a width 30 and a design height 24. The design height 24 generally corresponds to the height of the perimeter panel 12 for the cover into which the foam cushion 22 will be

inserted. The foam cushion 22 is generally the same dimensions as the cover into which it is inserted or very slightly larger than the cover. For example, a 4 inch, 1.4 pcf density foam cushion may be manufactured for a 4 inch finished cushion assembly height. As a result, the finished cushion assembly is virtually the identical shape and size, and perhaps slightly larger, as the manufactured dimensions of the foam cushion 22.

A manufactured fiber cushion 26 is illustrated in FIG. 3A. The manufactured fiber cushion 26 is constructed from a single layer of randomly oriented polyester staple fibers inter-linked to one another using a binder material, which is elastomeric in one example. In one example, the staple fiber and binder material are the same. The manufactured fiber cushion 26 includes a manufactured height 28 that is greater than a desired design finished height of the cushion 24. For example, if a finished height of 4 inches is desired, the manufactured fiber cushion 26 may be manufactured with 1.0 pcf of polyester fibers at a 5.6 inch height. The binder material is heated to a melting temperature to secure the staple fibers to one another once the melted binder material has solidified and produce a non-layered core batt. The core is compressed during its manufacture to provide a desired density, which is also affected by the staple and binder materials selected. The group of interlinked randomly oriented staple fibers 58 are shown schematically in more detail in FIG. 3B.

The individual staple fibers 52 include a fiber length 56 that is distributed in all three dimensions (x, y, z). In one example, the average fiber length 56 is approximately 2.5 inch. The manufactured height 28 is greater than the fiber length 56, which enables the fibers to be randomly distributed to the full extent of their fiber length in all three directions. This is contrasted with typical randomly oriented fiber manufacturing processes, such as cross lapping or air-laying, that orient the fibers in only two directions to form a relatively thin layer substantially less than the length of its staple fibers. Numerous cross lapped or air-layed layers are bonded in some fashion to one another to form a multi-layered fiber batt consisting of very thin layers. Fiber batts produced using an air-lay process do not make suitable cushions because they lose height over time to an unacceptable degree. The fiber batt formed according to this disclosure is typically an inch or greater in height, as opposed to the thin layers produced in air-lay processes, which are only fractions of an inch thick.

Referring to FIG. 4, the manufactured fiber cushion 26 is reduced from the manufactured height 28 to a tufted height 31 using one or more tufts 33, which may be rubber-like, for example. The tufts 33 include a body 37 extending between opposing heads 35, as illustrated in FIG. 6. The tuft 33 extends through the tufted cushion 36 to opposing surfaces 32. The width 30 of the tufted cushion 36 is generally the same as the width of the manufactured fiber cushion 26. Other tufting configurations can be used. For example, a lace and felt arrangement can be used, or a button and lace arrangement can be employed. Various tufting configurations can be used separately or in combination with one another for a given cushion assembly. The tuft 33 is not visible through the cover 11 with the cushion assembly 10 exposed and not otherwise in use. Thus, the presence of the tuft 33 is not apparent to an observer, which provides an aesthetically pleasing appearance.

The manufactured fiber cushion 26 includes a first density that is considerably less than the desired finished density of the cushion once placed within the cover. The cushion height is reduced from the manufactured height 28 to the tufted height 31, at least 5%, and in one example at least 10%, which increases the density from the manufactured fiber cushion 26

to the tufted cushion 36 at least 10%. In one example, if the desired finished height of the cushion within the cover is approximately 4 inches, the manufactured height 28 may be 5.6 inches, which when tufted and stuffed into a 4 inch high cover assembly 10 provides the comfort and resiliency of 1.4 pcf cushion that could not otherwise be provided by a 1.4 pcf cushion manufactured at a 4 inch height. Thus, the cushion will be reduced in height approximately 28%. In one example, the density is increased 40%. The example density of the manufactured fiber cushion 26 is 1.0 pcf for the 5.6 inch manufactured height.

An example tufted cushion 136 is illustrated in FIG. 5. The tufted cushion 136 includes a core 38 and topper layers 40 arranged on either side of the core 38 that are tufted together as an assembly. In one example, both the core 38 and the topper layers 40 are manufactured of three dimensionally randomly oriented polyester fiber inter-linked with one another as described above. The tufts extend through the core 38 and the topper layers 40. Other methods of attaching the core 38 and topper layers 40 can be used such as adhesive. The topper layers 40 may be constructed separately from the core 38, for example. Each topper layer is compressed during its manufacture to provide a desired density, which is also affected by the staple and binder materials selected. The topper layers 40 are of a lower density and different fiber blend than the core 38 to provide a desired hand and performance.

Referring to FIG. 7, the tufted cushion assembly 136 can be enclosed in a wrap 50, which provides functions like desired 30 flammability properties and/or hand, for example. The wrap 50 is arranged around the exterior surfaces of the tufted cushion 36, including the tufts 33 and provides an actual height 48 of the tufted cushion assembly 136. A perimeter height 42 is defined by the height of the perimeter panel 12. The perimeter 35 height 42 is approximately 90-98% of the actual or desired design height 24. The cover panels 14 provide a desired design height 44 (which should be very close to 24 and is determined by the cushion designer) and includes a crown or apex 46. The cover gradually increases to a location central to 40 the cover 11 to provide the apex. The desired design height 44 is greater than the perimeter height 42, and in one example at least approximately 120% of the perimeter height 42 at the apex 46. The cushion assembly 10 has a crowned surface or apex 46, whereas a cushion assembly using a foam cushion 45 has a generally flat or a nominal crown surface 60, illustrated in FIG. 8.

The disclosed cushion assembly and batt having randomly oriented staple fibers inter-linked to one another using a binder material is constructed with the following specifications:

Core:

density at manufactured height: 0.8-3.0 pcf, in one example, approximately 1.0 pcf  
manufactured thickness of 1.0-6.0 inch  
20-90 ILD

Topper:

density at manufactured height: 0.6-2.0 pcf  
manufactured thickness of 0.5-4.0 inch  
10-55 ILD

Cushion Assembly (Core and at Least One Topper Layer):  
density at desired design height, tufted: 1.0-3.0 pcf, in one example, approximately 1.4 pcf

support factor:  $\leq 3$ , with the ILD determined using a 4 inch batt at installed height, tufted

The performance of the batt can be increased by using more 65 binder and a higher denier fiber. Decreasing the amount of binder and using lower denier fiber decreases performance and cost. The binder and staple fibers for each layer are

**5**

selected to obtain the desired ILD for each layer in order to "tune" the overall cushion assembly. In one example, a tunable fiber cushion includes a batt of randomly oriented first polyester fibers interlinked with a first binder material. The batt has a non-layered core with a first manufactured height defined by opposing surfaces and that includes a first density. The first density is 0.8-3.0 pcf. At least one topper layer of randomly oriented second polyester fibers is interlinked with a second binder material. A topper layer includes a second manufactured height of a second density. The topper layer is arranged on a side adjacent to one opposing surface. The second density is 0.6-1.4 pcf. A tuft extends through the batt and the topper layer to provide a tufted cushion assembly having a tufted height and a third density at the tufted height that is greater than the first density or the second density. The third density is 1.0-3.0 pcf. The tufted cushion assembly at the tufted height provides a support factor of less than or equal to 3 with an ILD determined using a 4 inch batt sample of the tufted cushion assembly at the tufted height.

Although example embodiments have been disclosed, a worker of ordinary skill in this art would recognize that certain modifications would come within the scope of the claims. For that reason, the following claims should be studied to determine their true scope and content.

What is claimed is:

**1. A tunable fiber cushion comprising:**

a batt of randomly oriented first polyester fibers interlinked with a first binder material, the batt having a non-layered core made of a first fiber blend and defined by opposing surfaces;  
 at least one topper layer made of a second fiber blend of randomly oriented second polyester fibers interlinked with a second binder material, the at least one topper layer arranged on a side adjacent to one opposing surface, and wherein the second fiber blend is different from the first fiber blend;  
 a tuft extending through the batt and the at least one topper layer to provide a tufted cushion assembly having a tufted height and a density of 1.0-3.0 pounds per cubic foot (pcf); and

**6**

wherein the tufted cushion assembly at the tufted height provides a support factor of less than or equal to 3 with an Indentation Load Deflection (ILD) determined using a 4 inch batt sample of the tufted cushion assembly at the tufted height.

**2. The tunable fiber cushion according to claim 1, wherein the fibers include an average length are randomly oriented in three dimensions, the batt having a thickness that is greater than the average length to accommodate the average length in all three dimensions.**

**3. The tunable fiber cushion according to claim 1, wherein the at least one topper layer includes two topper layers arranged on opposite sides of the core adjacent respective opposing surfaces.**

**4. The tunable fiber cushion according to claim 1, comprising multiple tufts having a length generally corresponding to the tufted height and provided by a body having opposing heads, the heads abutting opposing surfaces of the cushion to retain the cushion at the tufted height.**

**5. The tunable fiber cushion according to claim 1, wherein the core and the at least one topper layer have different densities when at respective manufactured heights.**

**6. The tunable fiber cushion according to claim 5, wherein, when the core is at a manufactured height, the core has a first density of 0.8-3.0 pcf.**

**7. The tunable fiber cushion according to claim 6, wherein the density of the tufted cushion assembly is at least 110% of the first density.**

**8. The tunable fiber cushion according to claim 6, wherein the tufted height is less than approximately 90% of a sum of the manufactured height of the core and the manufactured height of the at least one topper layer.**

**9. The tunable fiber cushion according to claim 6, wherein, when the at least one topper layer is at a manufactured height, the topper layer has a second density that is less than the first density.**

**10. The tunable fiber cushion according to claim 9, wherein the second density is 0.6-2.0 pcf.**

\* \* \* \* \*